

Feb. 13, 1968

N. VOLIANIK

3,368,885

METHODS OF DESULPHIDING A BATH OF METAL

Filed Nov. 17, 1964



Fig. 2



Fig. 1

3,368,885

## METHODS OF DESULPHIDING A BATH OF METAL

Nicolas Volianik, Sevres, France; assignor to Centre Technique des Industries de la Fonderie, Paris, France, a 5  
public utility institute of France  
Continuation-in-part of application Ser. No. 128,515,  
Aug. 1, 1961. This application Nov. 17, 1964, Ser.  
No. 412,598  
Claims priority, application France, Aug. 18, 1960,  
836,083, Patent 1,274,499  
6 Claims. (Cl. 75—53)

### ABSTRACT OF THE DISCLOSURE

Molten metal is desulfurized by depositing powdered calcium carbide on the upper surface of the bath of molten metal and then blowing an inert gas into the bath below its surface at such a rate of flow as to cause violent turbulence in the bath producing eddies which draw the powdered calcium carbide from the upper surface and disperse it through the bath to effect rapid desulfurizing thereof. The operation takes but a few minutes and does not require heat to be applied to the molten metal to keep it molten.

This application is a continuation-in-part of my prior application Ser. No. 128,515, filed Aug. 1, 1961, and now abandoned.

The present invention relates to methods of desulfurizing a bath of metal, and has for an object, improvements therein.

It is known that a bath of metal may be desulfurized by depositing an alkaline oxide or carbonate on this bath and by agitating the whole by blowing in an inert gas such as nitrogen. However, this method can only be used if the bath of metal is contained in a container which has a neutral or basic coating, this condition being absolutely necessary to ensure the reproducibility of the rate of desulfurization and to prevent the coating from being attacked, an occurrence likely to happen if this coating were silico-aluminous.

It is also known that a metal bath may be desulfurized by the injection of calcium carbide with the aid of a gas such as nitrogen. In this case the vessel containing the bath can have an acid, basic or neutral coating. But the operation of this method is relatively complicated since it necessitates the use of injectors; besides this, it can become irregular in operation if the injectors become blocked.

Previous workers in the field have attempted to improve the desulphurization of liquid metal by blowing gas therethrough. For example, in U.S. Patent No. 2,587,573, Wynne discloses a system in which gas is bubbled through a melt in order to promote an agitation which serves to increase the desulphurization. However, this patent fails to disclose the velocity at which this gas passes into the bath and so the degree of agitation obtained cannot be determined. Moreover, Wynne discloses that with his process it was necessary to bubble gas through the melt for 70 to 120 minutes in order to obtain a satisfactory desulfurization. Such long treatment periods present obvious drawbacks, notably in that a large supply of gas must be used and, in particular for small masses of liquid metal, means must be provided to heat the metal so as to maintain it in a liquid state.

Applicant has discovered that all of these problems can be overcome if gas is bubbled into the melt at such a velocity as to cause a turbulence sufficient to produce eddies which are apparent at the surface of the liquid. No prior art process known to applicant suggests the produc-

tion of such a violent turbulence to enhance the desulphurization process.

This degree of turbulence is achieved by introducing the agitating gas into the melt at a velocity which is much higher than those used in the prior art. The result of this procedure is to reduce the time necessary to produce a satisfactory desulphurization (e.g., a reduction of the sulphur content of the melt by 80%) from the 70 to 120 minutes required by Wynne to a period of 3 to 5 minutes, and in some cases to as little as two minutes.

The advantages resulting from such a decrease in the desulphurization time include a reduction in the quantity of gas used, and the elimination of the need for auxiliary heating means for maintaining the melt in a liquid state.

It is therefore an object of this invention to radically decrease the time required for desulphurizing a mass of liquid metal.

It is another object herein to decrease the quantity of gas required in a process whereby desulphurization is accelerated by using a gas flow to agitate the liquid metal.

A still further object of this invention is to eliminate the need for auxiliary heating equipment to maintain a mass of metal in its liquid state during a desulphurizing process.

The present invention has for another object a method of desulfurizing a bath of metal the operation of which is very simple and can be carried out in a vessel with any type of covering which allows very high and regular rates of desulfurization to be obtained.

The method according to the invention essentially consists in depositing at one time all the required powdered calcium carbide directly on the surface of the bath, the granulation of the powder being preferably comprised between 0.5 and 1 millimeter and in agitating very energetically by blowing in a gas by means of one or more tubes through one or more openings situated below the surface of the metal, arranged so as to bring about a random turbulence of the liquid metal. In this manner and with a particularly simple apparatus, all of the calcium carbide particles are literally enveloped, almost instantaneously, by the eddies brought about on the surface of the bath by the turbulence of the liquid metal, thus ensuring, by the intimate contact between the metal and the calcium carbide, the speed and efficiency of their reaction. They cannot become separated from the bath by a gaseous envelope as is the case with the injection-desulfurizing processes.

This turbulence, which becomes evident at the surface of the bath, must not become a regular movement of the liquid metal which would simply have as its effect to renew the particles of liquid metal in order to put them successively into contact with the calcium carbide which would remain on the surface; it must cause eddies such that the carbide is driven into the middle of the bath and regularly distributed within the liquid mass.

To this end the gas must be blown in through one or more tubes having openings of a section of the order of a square centimeter without any diaphragm, porous stoppers or any other regulating device being inserted.

The gas to be used may be an inert gas such as nitrogen or argon, but air may be used since, when calcium carbide is used, oxygen will not change the chemical composition of the molten metal.

The velocity with which gas must be blown into the melt in order to produce the required degree of turbulence does not have a unique value for all cases, but varies according to the quantity of metal being treated. However, the velocity required to achieve, for example, an 80% reduction in the sulphur content of the metal within a period of 3 to 5 minutes can be expressed as a linear function of the quantity of metal being treated.

This function may be given as:

$$V \geq 9T + 30 \quad (1)$$

where

V equals the velocity of the gas in meters/sec. as it leaves its tube, and

T equals the quantity of metal being treated, in tons (1 ton = 2200 lbs.).

It should be understood that this equation is not intended to be limiting inasmuch as the velocity could be slightly lower and still produce the improved results described herein. It must also be noted that the process hereunder discussion is intended to be carried out with the melt at a temperature of at least 1350° C. and using a quantity of calcium-carbide which is between 0.009T and 0.015T (where T is the quantity of melt in tons).

When a gas introduction tube or tubes having an opening of the order of a square centimeter are used, the volumetric flow rate of the gas for each tube can be expressed by the relation:

$$Q = \frac{V}{3} \quad (2)$$

where Q is in m.<sup>3</sup>/hour.

These relations clearly show that both the gas velocities and the volumetric flow rates are far greater than those employed in similar prior art processes.

The most significant differences presented by the present process may clearly be seen from the following table comparing the values of various parameters according to the present process with those of similar parameters according to Wynne's process. It should be mentioned that inasmuch as the Wynne patent fails to set forth the dimensions of his gas introduction pipe, the cross section thereof was assumed to be 1 cm.<sup>2</sup>. All of the remaining figures were taken directly from the patent.

TABLE I

|                                                               | 190 lbs. of melt |          | 13.6 tons of melt |          | 31.7 tons of melt |          |
|---------------------------------------------------------------|------------------|----------|-------------------|----------|-------------------|----------|
|                                                               | Wynne            | Volianik | Wynne             | Volianik | Wynne             | Volianik |
| Volumetric rate of gas-flow per ton of melt (liters/min./ton) | 20               | 2,700    | 14                | 185      | 15.7              | 165      |
| Actual flow rate (m. <sup>3</sup> /hour)                      | 0.08             | 10.2     | 11.32             | 152.5    | 29.7              | 315      |
| Gas exit velocity (M/sec.)                                    | 0.22             | 30.5     | 10.5              | 152.5    | 27.5              | 315      |
| Duration of process (min.)                                    | ≤90              | ≤4       | ≤90               | ≤4       | ≤90               | ≤4       |
| Quantity of gas consumed (m. <sup>3</sup> )                   | 0.12             | 0.68     | 17                | 10.16    | 44.6              | 21.0     |

#### Comparison between present process and that of Wynne

This table clearly shows the distinctly lower gas flow rates and velocities (assumed) used by Wynne, which values have been found to be clearly incapable of inducing the eddy-producing turbulences characteristic of the process of the present invention.

Insofar as concerns the number of tubes used in the practice of the present process, it has been discovered that satisfactory results will be obtained when using one tube for masses of liquid metal weighing less than one ton and three tubes for larger masses. These tubes may preferably be submerged to a depth of 20 to 30 cm. above the bottom of the liquid container.

When the flow rates and velocities are chosen according to Equations 1 and 2 above, one may determine the approximate duration of treatment and percentage of CaC<sub>2</sub> (with respect to the weight of metal treated) required to reduce the sulphur content of the metal by 80%, according to the following equations:

$$\text{Duration (minutes)} \geq 17.9 - 0.01\theta \quad (3)$$

$$\text{Percent CaC}_2 = \frac{\text{Weight of CaC}_2}{\text{Weight of metal}} \times 100 \geq 7 - 0.004\theta \quad (4)$$

where  $\theta$  equals the temperature of melt in degrees centigrade at the start of the process.

Another feature of the present invention resides in the fact that the powdered calcium carbide is deposited on the surface of the bath only after the molten metal has been poured into its treatment vessel, whereas previous experimenters have taught that the powdered desulfurizing agent should be placed on the bottom of the vessel prior to the pouring of the molten metal. Applicant's novel procedure represents a distinct improvement because it permits the addition of exactly the quantity of calcium carbide needed after the quantity of metal in the vessel has been determined and because it permits the molten metal to be deslagged prior to the addition of the calcium carbide, thus further ensuring an intimate contact between the latter and the metal.

The method according to the invention leads to surprising results, particularly regarding the high degrees of desulfurization obtained and the speed of the operation which does not normally exceed 2 to 3 minutes.

Now, this operational speed is essential in order to prevent the bath from cooling. Moreover, the treatment container or crucible may with advantage be heat-insulated in order to slow down this cooling process.

The invention will now be described with reference to the following specific examples.

#### Example 1

800 kilograms of a liquid fount having a sulphur content of 0.09% were melted in a container. 8 kilograms of calcium carbide were scattered on the surface of the bath and nitrogen bubbled through at a velocity exceeding 37 m./sec. with the aid of one tube immersed in the bath, for a duration of two minutes. It was then found that the sulphur content was 0.027%, i.e. had been lowered by 70%.

#### Example 2

800 kilograms of a liquid fount having a sulphur con-

tent of 0.08% were melted in a container. 11.2 kilograms of calcium carbide were scattered on the surface of the bath and nitrogen bubbled therethrough for three minutes at a velocity exceeding 37 m./sec. It was then found that the sulphur content was 0.006%, i.e. had been lowered by 92.5%.

The accompanying drawings illustrate by way of example two embodiments of apparatus for performing the invention.

FIG. 1 is a diagrammatic illustration of the principle involved.

FIG. 2 shows an embodiment of a more commercial character.

In FIG. 1 there is shown at 1 the ladle or crucible in which a bath of molten cast iron is contained. Dipping into this bath is a tube 2 connected by a collar 3 with a bent rigid tube 4 which in turn is connected through a flexible tube 5 and a flowmeter 6, to a container of compressed gas 7, such as nitrogen or air.

In the embodiment of FIG. 2, the ladle or crucible is again shown at 1, the compressed gas container at 7, and the flow meter device at 6. This device itself is connected to the container 7 through an intermediate tube 8 and a pressure reducer valve 9. Three graphite tubes 2 are here provided and are carried from a common support 10 provided with a clamping arrangement 11, the support 10 being in turn secured to one end of the piston

rod 12 of a ram actuator 13 carried by a fixed bracket 14 above the crucible 1. The respective tubes 2 are connected through tubes 15 with a feeder head 16 connected by a common flexible pipe 17 with the container and flowmeter 6. The tubes 15 finally are connected at 19 with the tubes.

Further in this figure there is shown at 18 a hollow union for assembling two adjacent tube elements 2. The ram 13 provides the possibility of controlling at will the downward and upward movements of the tubes 2 into the ladle and crucible and thereby accurately determining the duration of the process.

It will be understood that the apparatus may admit of a large number of modified embodiments, particularly as concerns the means for raising and lowering the tubes.

I claim:

1. A method of desulfurizing a bath of molten metal, comprising the steps of depositing powdered calcium carbide on the top surface of said bath, and blowing a gas into said bath below the surface thereof, for a period not exceeding 10 minutes, through at least one opening having an unobstructed cross sectional area of the order of 1 cm.<sup>2</sup> at a rate of flow sufficient to cause violent turbulence in said bath producing eddies which draw the powdered calcium carbide from said top surface and disperse the same throughout the bath for ensuring the rapid desulfurizing of all the molten metal prior to cooling of the latter.

2. A process as recited in claim 1, wherein said calcium carbide consists of particles in the size range between approximately 0.5 and 1.0 mm.

3. A process as recited in claim 1, wherein said gas is blown into said bath for a period not exceeding 5 minutes.

4. A process as recited in claim 1 wherein said gas is introduced into said bath at a velocity in meters per second which is numerically superior to six times the quantity of molten metal being treated, in tons, plus ten meters per second.

5. A method of desulfurizing a bath of molten metal, comprising the steps of depositing powdered calcium carbide on the top surface of said bath, and blowing a gas into said bath below the surface thereof and at a velocity V, in meters per second, superior to  $6T+10$  where T is the quantity of molten metal being treated, in tons, through at least one unobstructed opening at a rate of flow sufficient to cause violent turbulence in said bath for producing eddies which draw the powdered calcium carbide from said top surface and disperse the same throughout the bath for ensuring the rapid desulphiding of all of the molten metal prior to cooling of the latter.

6. A process according to claim 5 wherein said calcium carbide is deposited directly on the top surface of said molten metal after the latter has been poured into its treatment vessel.

#### References Cited

#### UNITED STATES PATENTS

2,577,764 12/1951 Hulme ----- 75-93 X

DAVID L. RECK, *Primary Examiner.*

HYLAND BIZOT, *Examiner.*

N. P. BULLOCH, H. W. TARRING,

*Assistant Examiners.*